

Dec. 1, 1953

A. L. STILLMAN

2,661,326

METHOD OF MANUFACTURING BRIQUETTES

Filed April 5, 1948



INVENTOR  
Albert Leeds Stillman

BY

*Klein & Hart*

ATTORNEYS

## UNITED STATES PATENT OFFICE

2,661,326

METHOD OF MANUFACTURING  
BRIQUETTES

Albert Leeds Stillman, Plainfield, N. J., assignor to  
Fuel Research Corporation, New York, N. Y., a  
corporation of Delaware

Application April 5, 1948, Serial No. 19,160

2 Claims. (Cl. 202—25)

1

This invention relates to the manufacture of briquettes, and more particularly to improvements in the production of smokeless coal briquettes.

The primary purpose of the invention is to provide a process by which a smokeless, rapidly and evenly burning briquette of convenient size can be made in an inexpensive manner.

The briquette of this invention is composed of finely powdered coal, preferably a bituminous or semi-bituminous coal which ordinarily would swell when heated, such as those coals known as Pocahontas and Lower Kittanning. The coal is first heated in a drying apparatus at a temperature of not less than 350 degrees F. and not more than 400 degrees F. for a period of about ten minutes, and then is cooled at atmospheric temperature. As a result of this treatment, the swelling quality of the coal is practically eliminated. The coal is then ground finely so that the whole passes through a sieve of from 60 to 200 meshes per linear inch.

The thus treated coal may be utilized as the carbonaceous matter of the briquette, or the latter may be composed of a mixture of such coal and pitch, or a mixture of such coal, pitch and lignous material. It is preferred that the carbonaceous matter of the briquette include from 5 to 10% by weight, of a mineral pitch, such as oil asphalt (also called refiner's waste) having a melting point of approximately 300 degrees F. The pitch or asphalt is first ground to pass wholly through a sieve of from 60 to 200 meshes per linear inch, and then mixed in any suitable fashion with the heat treated, ground coal. It is also preferred that the carbonaceous matter of the briquette include approximately 15% by weight, of lignous material, such as sawdust or ground sugar cane waste. This material may be added with the pitch to form the mixture or may be intermixed with the mixture of coal and pitch.

Whether the finely ground carbonaceous material be composed wholly of coal, or a mixture of coal and pitch, or a mixture of coal, pitch and lignous material, such material is then placed in a receptacle divided by partitions into a plurality of compartments or cells. The receptacle is preferably a rectangularly-shaped open receptacle about two inches high and divided into compartments or cells of about four square inches in area; the top edges of the partitions being flush with the top edges of the receptacle. The material of the receptacle as well as the partitions thereof, is made of combustible material, such as wood or paper. In filling the

2

compartments or cells of the receptacle, sufficient of the carbonaceous material is inserted therein so that it will be flush with the top edges of the receptacle and its partitions. In other words, the compartments or cells are completely filled with the carbonaceous material. The filled receptacle is then placed in a closed retort and heated in the latter under lowered vapor tension obtained by pumping out the atmosphere in the retort by means of a pump. The retort is externally heated to a temperature of approximately 1000 degrees F. and the filled receptacle is subjected to such temperature in the retort for about one hour or until the gases have been sufficiently driven from the carbonaceous material as to render it practically smokeless. At the end of that period, the carbonaceous material will have carbonized into rectangular shapes of the compartments and the material of the receptacle will have carbonized into a fragile carbon so that the whole mass may be readily broken into rectangularly-shaped briquettes of convenient size for burning and handling.

The principal steps of the above described method in the form of a flow sheet are shown on the accompanying drawing.

It will be noted from the foregoing that the briquette of this invention is composed of from about 75% to approximately 100% of carbonized coal and that portion of the fragile carbon resulting from the receptacle and adhering to the carbonized carbonaceous material in the briquette when the carbonized mass is broken up into briquettes. As has previously been mentioned, the coal may be either of the bituminous or semi-bituminous type, hence, where in the appended claims reference is made to "bituminous coal," it is to be understood that such term also includes semi-bituminous coals. The purpose of preheating the coal at a temperature of from 350 degrees to 400 degrees F. is to prevent any danger of the coal breaking the partitions of the receptacle during the carbonizing step. As a further result of such preheating treatment and the carbonizing of the carbonaceous material in the retort, a large part of the non-flammable gases in such material is driven off, thereby enabling the finished briquettes to be lighted readily, to burn evenly and completely, and to be easily tended. These qualities of the briquette are enhanced by the presence of the lignous material which lightens the briquette and increases its friability. The process of making the briquettes of this invention is simple and inexpensive and obviates the necessity of using

presses such as are now employed in practically all briquetting plants and which add materially to the cost of manufacturing this product. Furthermore, by reason of the fact that the receptacle or briquette mold itself is transformed into a fragile carbon forming part of the briquettes, the expense of handling the product is reduced to a minimum.

I claim:

1. The method of manufacturing briquettes, which comprises subjecting a bituminous coal which ordinarily would swell when heated, to a temperature of from 350 degrees F. to 400 degrees F. for ten minutes, cooling the thus treated coal to atmospheric temperature, grinding the treated coal until it passes wholly through a sieve of 60 mesh, mixing with the coal ground mineral pitch and ligneous material to form a finely powdered carbonaceous material in which the pitch forms approximately 5% to 10% by weight, of such carbonaceous material, the lignous material forms approximately 15% by weight, of such carbonaceous material, and the ground, treated bituminous coal forms approximately from 75% to 80% by weight, of such carbonaceous material, filling a receptacle made of solid cellulose material and composed of a plurality of small compartments with the powdered carbonaceous material, and then subjecting the filled container to a temperature of approximately 1000 degrees F. in a closed retort under lowered vapor tension until the carbonaceous material has been converted into carbonized low temperature char and the cellulose material of the receptacle has been transformed into layers of fragile carbon on the surfaces of the briquettes.

2. The method of manufacturing briquettes, which comprises heat treating a bituminous coal to eliminate any substantial tendency to swell, grinding the thus treated coal until it passes

wholly through a sieve of 60 mesh, mixing with the coal approximately 5% to 10% by weight, of ground mineral pitch to form a finely powdered carbonaceous material, the ground bituminous coal being mixed with the ground pitch in sufficient quantity to form approximately from 75% to 80% by weight of the carbonaceous material, mixing with the coal and pitch, approximately 15% by weight, of lignous material, filling a receptacle made of solid cellulose material and composed of a plurality of small compartments with the powdered carbonaceous material, and then subjecting the filled container to a temperature of approximately 1000 degrees F. in a closed retort under lowered vapor tension until the carbonaceous material has been converted into carbonized low temperature char and the cellulose material of the receptacle has been transformed into layers of fragile carbon on the surfaces of the briquettes.

ALBERT LEEDS STILLMAN.

References Cited in the file of this patent

UNITED STATES PATENTS

| Number    | Name     | Date          |
|-----------|----------|---------------|
| 415,734   | Randall  | Nov. 26, 1889 |
| 1,481,942 | Vogel    | Jan. 29, 1924 |
| 1,561,322 | Goskar   | Nov. 10, 1925 |
| 1,593,208 | Culmer   | July 20, 1926 |
| 1,618,248 | Walton   | Feb. 22, 1927 |
| 1,772,053 | McIntire | Aug. 5, 1930  |
| 2,105,832 | Becker   | Jan. 18, 1938 |
| 2,158,666 | Otto     | May 16, 1939  |
| 2,314,641 | Wolf     | Mar. 23, 1943 |
| 2,341,861 | Fuchs    | Feb. 15, 1944 |

FOREIGN PATENTS

| Number  | Country       | Date          |
|---------|---------------|---------------|
| 279,020 | Great Britain | Dec. 22, 1927 |
| 499,432 | Great Britain | Jan. 24, 1939 |